

## UNITED STATES PATENT OFFICE

GEORGE RIVAT, OF PATERSON, ERNEST CADGÉNE, OF ENGLEWOOD CLIFFS, NEW JERSEY, AND CAMILLE DREYFUS, OF NEW YORK, N. Y., ASSIGNORS TO CELANESE CORPORATION OF AMERICA, A CORPORATION OF DELAWARE

## DYEING OF CELLULOSE DERIVATIVES

No Drawing.

Application filed June 30, 1926. Serial No. 119,742.

The object of this invention is to provide a process of fixing iron salts on or in materials containing organic derivatives of cellulose. Another object of this invention is to provide a process for fixing iron salts on or in materials containing organic esters of cellulose, more particularly cellulose acetate. Still another object of the invention is to provide a process for treating materials containing organic derivatives of cellulose so that they may be dyed more easily and with more satisfactory results than has heretofore been possible.

It is customary when it is desired to mordant silk, etc., with iron salts, that an iron salt solution of 1 to 5% strength be used. This process when applied to materials containing organic esters of cellulose, results in no appreciable fixation of iron in the material. The applicants have now discovered that if material containing organic esters of cellulose is treated with a highly concentrated solution of iron salts, appreciable amounts of the iron are easily fixed in or on the cellulose derivative treated. The strength of the iron salt solution should be between 40 to 55% by weight in order to obtain good results.

As an example of the operation of the process the following is given:  
A fabric made from cellulose acetate was treated in a 50% bath of ferric chloride for one hour. The bath was first heated to 40 degrees centigrade which was gradually increased to 60 degrees centigrade. The material was then squeezed or whizzed to remove the excess of the iron solution, after which it was washed in water for twenty minutes. After this washing the material was again washed, this time in cold water containing 1 c. c. of ammonia per litre of water.

The fabric after the above treatment was orange colored but was unchanged in other respects. It still retained its lustre and its softness. The iron was permanently fixed in the cellulose acetate and could not be removed even when the material was treated with hydrochloric acid. The fabric treated as above when washed was found to contain 1.8-2% of iron.

The applicants have discovered that a fab-

ric which has been subjected to the above treatment can be dyed with the so-called natural or vegetable dyes. When such fabrics are dyed with this class of dyes unexpected results are obtained. The colors are very fast and deep whereas similar fabrics when untreated do not dye at all well with this class of dyes.

Thus when a cellulose acetate fabric which was first treated with ferric chloride, washed, etc., as set out above, was immersed in a regular log-wood black bath in soap, say at a temperature of 70° C., for one hour it was found to have been dyed a beautiful black, much superior in appearance to that previously obtainable with this dye.

Where a mixed fabric of cellulose acetate and silk, or cellulose acetate and wool or of cellulose acetate, silk and wool, was treated in accordance with this process a very unusual and desirable result was noticed. The silk or wool when treated as above and then dyed in a logwood black bath as stated, was found to have been dyed the same shade as was the cellulose acetate. This results in a very great saving of time, labor and expense, since the mixed fabric does not have to be passed thru two or three different dye baths, as is the practice today. What has been said above with respect to the logwood dyeing of the organic derivatives of cellulose is also true of other natural or vegetable dyes or dye extracts such as, for example, young fustic, fustic, quercitron, Persian berries, weld extract, turmeric, sandalwood, cutch, etc. or any other dyes or mixtures of dyes which are suitable for dyeing a material mordanted with iron. The choices of dyes will depend upon the color which it is desired to dye the material. In all cases after the dyeing the goods must be washed as is customary in similar ordinary dyeing processes.

In the event it is desired to tint the black obtained by the logwood dyeing either bluer or greener, this can be accomplished by adding the proper dyestuffs to the logwood bath. For the cellulose acetate fabric an SRA dyestuff (that is a water insoluble dyestuff having an affinity for cellulose acetate material and generally applied in the form of an

aqueous dispersion obtained for instance with the aid of a dispersing agent) may be used whereas a basic dyestuff may be employed to tint real silk if it is present and an acid dyestuff for wool. The above examples are merely illustrative and merely set out a few of the numerous possible methods of carrying out the applicants' invention. Thus the ferric chloride can be replaced by any other soluble ferric salt such as, for instance, ferric sulphate, ferric nitrate, etc. Also the cellulose acetate can be replaced by cellulose propionate, cellulose butyrate, ethyl cellulose, etc. and, as stated above, logwood may be replaced by fustic or other dyes as stated above.

This process is applicable not only to materials made wholly of organic derivatives of cellulose but can also be utilized to treat mixtures of such derivatives and other materials such as, for example, mixtures of cellulose acetate and wool, cellulose acetate and silk, and cellulose acetate and wool and silk with very desirable results. The treatment of such mixtures, however, is to be considered within the scope of this invention.

Having described our invention what we desire to claim by Letters Patent is:

1. A process of treating organic derivatives of cellulose which comprises subjecting the same to the action of a concentrated solution of a ferric salt.

2. A process of treating organic derivatives of cellulose which comprises subjecting the same to the action of a 40 to 55% solution of ferric chloride.

3. A process of treating organic esters of cellulose which comprises subjecting the same to the action of a concentrated solution of a ferric salt.

4. A process of treating organic esters of cellulose which comprises subjecting the same to the action of a 40 to 55% solution of ferric chloride.

5. A process of treating organic esters of cellulose which comprises subjecting the same to the action of a 50% solution of ferric chloride.

6. A process of treating organic esters of cellulose which comprises subjecting the same to the action of a concentrated solution of ferric chloride at temperatures above atmospheric and below 60° C.

7. A process of treating organic esters of cellulose which comprises subjecting the same to the action of a 50% solution of ferric chloride for approximately one hour at 40 to 60° C.

8. A process of treating organic esters of cellulose which comprises subjecting the same to the action of a 50% solution of ferric chloride for approximately one hour at 40 to 60° C. removing the excess iron chloride solution, then washing the material with

warm water and finally washing it with cold water containing ammonia.

9. A process of treating cellulose acetate which comprises subjecting the same to the action of a concentrated solution of a ferric salt.

10. A process of treating cellulose acetate which comprises subjecting the same to the action of a concentrated solution of ferric chloride.

11. A process of treating cellulose acetate which comprises subjecting the same to the action of a 50% solution of ferric chloride.

12. A process of treating cellulose acetate which comprises subjecting the same to the action of a 50% solution of ferric chloride. for approximately one hour at 40 to 60° C.

13. A process of treating cellulose acetate which comprises subjecting the same to the action of a 50% solution of ferric chloride for approximately one hour at 40 to 60° C. removing the excess iron chloride solution, then washing the cellulose acetate with water and finally washing it with cold water containing ammonia.

14. A process of treating organic esters of cellulose which comprises subjecting the same to the action of a concentrated solution of a ferric salt, removing the excess ferric salt solution, then washing the material with warm water, again washing with cold water containing ammonia, and then treating the thus washed material with a dye extract and then finally washing the dyed material as usual.

15. A process of treating organic esters of cellulose which comprises subjecting the same to the action of a 50% solution of ferric chloride removing the excess ferric chloride solution, then washing the material with water, again washing with cold water containing ammonia, and then treating the thus washed material with a natural dye extract and then finally washing the dyed material as usual.

16. A process of treating cellulose acetate which comprises subjecting the same to the action of a 50% solution of ferric chloride for approximately one hour at 40 to 60° C., removing the excess ferric chloride solution, then washing the acetate with warm water, again washing, with cold water containing ammonia, then treating the thus washed material with a natural dye extract and finally subjecting the dyed material to the usual washing operations.

17. A process of treating cellulose acetate which comprises subjecting the same to the action of a 50% solution of ferric chloride for approximately one hour at 40 to 60° C., removing the excess ferric chloride solution, then washing the acetate with water, again washing, with cold water containing ammonia, then treating the thus washed material with logwood extract and thereafter

70

75

80

85

90

95

100

105

110

115

120

125

130

subjecting the dyed material to the usual washing operations.

18. A process of treating cellulose acetate which comprises subjecting the same to the action of a 50% solution of ferric chloride for approximately one hour at 40 to 60° C., removing the excess ferric chloride solution, then washing the acetate with water, again washing with cold water containing ammonia, then treating the thus washed material with the regular logwood black bath in soap for one hour at approximately 70° C.

19. A process of treating a mixed fabric containing wool and cellulose acetate which comprises subjecting said fabric to the action of a 50% solution of ferric chloride for approximately 1 hour at 40 to 60° C.

20. A process of treating a mixed fabric of wool and cellulose acetate which comprises subjecting said fabric to the action of a 50% solution of ferric chloride for approximately 1 hour at 40 to 60° C., removing the excess ferric chloride solution, then washing the fabric with water, again washing with cold water containing ammonia, then treating the thus washed fabric with logwood extract and thereafter subjecting the dyed fabric to the usual washing operations.

21. Cellulose acetate having 1.8-2% of iron fixed therein by treating the cellulose acetate with a 50% solution of ferric chloride.

22. Cellulose acetate having 1.8-2% of iron fixed therein and dyed with logwood extract thereon.

23. A mixed fabric containing wool and cellulose acetate having 1.8-2% iron fixed therein.

In testimony whereof, they have hereunto subscribed their names.

GEORGE RIVAT.  
ERNEST CADGÉNE.  
CAMILLE DREYFUS.